

# UNITED STATES PATENT OFFICE.

LOUIS SAPERY, OF BROOKLYN, NEW YORK.

## BABBITT-METAL PRODUCT AND PROCESS OF MAKING SAME.

Specification of Letters Patent. Patented Aug. 31, 1920.

1,351,404.

No Drawing.

Application filed May 21, 1920. Serial No. 383,315.

*To all whom it may concern:*  
Be it known that I, Louis SAPERY, citizen of the United States of America, residing at 1370 Carroll St., Brooklyn, N. Y., in the county of Kings and State of New York, have invented certain new and useful Improvements in Babbitt-Metal Products and Processes of Making Same, of which the following is a specification.

10 The present invention relates to putting up Babbitt metal in a novel form, whereby its usefulness is considerably enhanced, and the invention is applicable to the treatment of various kinds of babbitt. Babbitt metal is usually put up and sold in the form of bars of convenient size, and when the same is to be employed by the consumer, one or more of the bars are placed in a pot and heated until the same melts, after which it 15 is cast into the desired form; for example, it is cast into a casing of a journal box. During the time that the Babbitt metal is held in the pot on a molten condition, it has a tendency to absorb more or less oxygen from the air, which oxidizes some of the 20 metals present in the babbitt and, at any rate, the absorption of oxygen by the molten babbitt is found to substantially deteriorate its properties and the properties of 25 the resulting casting. In accordance with 30 the present invention, it has been found that the absorption of oxygen can be reduced to a great extent, if the bars of Babbitt metal after cooling are plated with 35 a metal which has a much higher melting point than the babbitt and which does not readily melt, and which is not readily taken up by the molten babbitt, but which forms 40 a layer of unmelted metal on the top of the layer of molten babbitt.

As examples of metals capable of producing the desired result, nickel and copper are mentioned as being particularly suitable. These metals can readily be applied to the 45 bars of babbitt by an ordinary electro-plating process, and the coating of the protective metal on the bars of metal may be quite thin, say, about one-thousandth of an inch in thickness.

50 While electro-deposition or electro-plating of copper and nickel upon various base metals has been known for a long time, it has not been heretofore recognized that Babbitt metal could be improved and its 55 usefulness substantially enhanced by elec-

tro-plating or otherwise applying a thin coating of such metals to the surface of the bars of babbitt.

Without limiting the invention thereto, it is stated for the purpose of illustration, 60 that the coating of a babbitt composed of 75% lead, 15% antimony, 10% tin, with an electro-plating of copper, of about .001 inch thickness has given good results. Also the similar application of nickel has given good 65 results. However, a coating substantially less than .001 inch in thickness has been found to give satisfactory results. A coating that is .001 inch in thickness has been found to give excellent results in all tests. 70

The nature of the metal that forms the thin film or coating is not without importance. The metal must be such as will have no deleterious effect upon the bearing qualities of the babbitt. Any metal which would 75 have a substantially deleterious effect upon the babbitt is excluded from consideration in connection with this invention. Copper and nickel have been found best adapted for use in forming the coating on the bar of 80 Babbitt metal.

The action of the film or coating of copper (or like metal) may be described as follows: The Babbitt metal is generally in the form of small flat bars or slabs which weigh approximately five pounds. The coating or film that is deposited on the flat bar by electro-plating covers the surface of the bar but forms no part of the Babbitt-metal alloy. As a rule, the bars are not 90 broken into pieces before being put in the melting-pot, unless the metal-worker does not wish to melt down as much as five pounds of Babbitt metal; but the bars are thrown into the melting-pot whole. Since 95 the Babbitt metal fuses at a much lower temperature than the metal of the electro-plated film or coating, this coating remains unfused and floats upon the surface of the molten Babbitt metal, which is of high 100 specific gravity due to its content of lead. The metal of the electro-plated coating is tough from which it results that the latter does not break up but remains intact and is borne on the surface of the molten Babbitt metal in much the same manner as waxed paper rests upon the surface of a vessel of water. Naturally, if there is considerable or violent disturbance of the molten mixture, the tough film of copper may become 110

disintegrated. Even though the area of the surface of the molten mixture may become, due to the expansion of the Babbitt metal as heat is applied thereto, greater than the 5 area of the film or plating, yet sufficient of the surface of the molten mixture is covered to protect the Babbitt-metal ingredients in a very substantial manner from oxidation and the mixture from deterioration or lowering 10 in quality due thereto. This invention is particularly useful in connection with lead-based babbitts or babbitts the tin content of which is relatively small. Tin gives tensile strength to Babbitt metal and it is likely to 15 become oxidized; and, where the tin content is small, oxidation thereof even to the extent of a small proportion of the whole results in a serious lowering of the quality of the Babbitt metal. Many metal-workers melt 20 down their babbitts without using a thermometer and the result is an overheating of the mixture; and the film or plating will prove particularly effective in preventing a loss of the tin content due to oxidation,

when such overheating is permitted to 25 occur.

I claim:

1. The process of protecting Babbitt metal from oxidation while being melted, which consists in coating the Babbitt metal, 30 prior to melting the same, with a thin film of another metal which is without injurious action on the bearing qualities of the Babbitt metal and which has a melting point that is substantially higher than that of the 35 Babbitt metal.

2. Babbitt metal coated with a thin film of another metal which is without injurious action on the bearing qualities of the Babbitt metal and which has a melting point 40 that is substantially higher than that of the Babbitt metal which it coats.

In testimony whereof I hereunto affix my signature in the presence of two witnesses.

LOUIS SAPERY. [L. S.]

Witnesses:

A. HOYT LEVY,

PETER J. KIERNAN.